

(Specimen.)

J. G. STEPHENS.

FIBER FOR UPHOLSTERY PURPOSES.

No. 283,161.

Patented Aug. 14, 1883.

Fig. 1.



Fig. 2.



Fig. 3.



Fig. 4.



Fig. 5.



WITNESSES:

Benj. A. Dare  
O. Gilligan.

INVENTOR.

John George Stephens.  
BY J. P. Thayer.

ATTORNEY

# UNITED STATES PATENT OFFICE.

JOHN GEORGE STEPHENS, OF BROOKLYN, ASSIGNOR TO CHARLES V. WARE,  
OF NEW YORK, N. Y.

## FIBER FOR UPHOLSTERY PURPOSES.

SPECIFICATION forming part of Letters Patent No. 283,161, dated August 14, 1883.  
Application filed July 19, 1882. (Specimens.)

*To all whom it may concern:*

Be it known that I, JOHN GEORGE STEPHENS, a subject of the Queen of Great Britain, and residing at Brooklyn, Kings county, New York, 5 have invented new and useful Improvements in Fiber for Upholstery Purposes, of which the following is a specification.

My invention consists of a new article of manufacture for upholstery purposes, the same 10 being natural vegetable fiber or animal-hair curled, rubbed, pressed, and fixed or set in the curled form by the effect of heat, rubbing, pressure, and coiling around a mandrel, the 15 fibers being fixed and permanently set substantially in the form of concentric rings or curls, as distinguished from spiral coils of the roped fibers.

Fiber twisted by the roping process has to be moistened and twisted in the moistened 20 state, to enable it to take the set of the twist so as to retain the curl after being picked apart. The long time required to dry it in the damp twisted state is damaging to the fiber, and the twisted coils are difficult to pick and 25 damaging to the fiber. The crimped fiber is better; but from the short time that it is subject to the pressure in the crimping-rolls and the lack of rubbing action during such pressure, such fiber fails of the requisite stiffness, 30 permanence of the set, and rigidity of the fiber desirable for the better qualities of upholstery goods. I therefore propose to make fiber for such purposes that is curled instead of twisted, as by the roping process, or crimped, 35 as by the crimping process, and that is set in the curls for stiffness thereof and for stiffness in the fiber by rubbing and pressure and heat in the curling process, the said curled, rubbed, and pressed fiber being much more permanent 40 in the curls and in the stiffness of the fiber itself than any now in use.

The superiority of my improved manufactured fiber, as compared with the crimped fiber heretofore prepared by me, consists in 45 the greater rigidity, more permanent set, and higher polish imparted to it by the longer retention of it in the form in which it is shaped by the devices employed therefor, and by the longer and more efficient heating to which it is 50 subject, and it is by these properties that it

may be distinguished from such fiber and also from hair curled by the roping process, which, besides being less rigid in the set, is softer in the fiber and lacking in the polish imparted to my fiber by the pressure, heat, and rubbing. 55 My improved fiber is also distinguished from shredded or artificial fiber which has been curled by roping, in that it consists of natural fibers only, the shredded fiber being incapable of sustaining the rubbing process essential 60 to the production of my improved fiber.

Figure 1 in the accompanying drawings is a sectional elevation of feeding, curling, rubbing, and pressing apparatus that may be employed in producing the improved fiber of my 65 invention. Fig. 2 is a plan view of the said apparatus. Figs. 3 and 4 are perspective views 70 of coils or bunches of the curled, rubbed, and pressed fiber as it is delivered from the machine; and Fig. 5 is a side elevation of a bunch of the said improved fiber when picked from the cocoon-shaped bunches of Figs. 3 and 4 as they come from the machine.

I employ a steam or gas heated rotary spindle, *a*, preferably a little conical in form, a 75 steam-heated rubbing-trough, *b*, feeding-rollers *c*, and any suitable chute, *d*, through which I run the fiber *e*, coiling it on the spindle, beginning at the point and moving the chute *d* slowly along the rods *f* to the base or bearing 80 supports of the spindle, so that it draws and winds the fibers snugly around it, and rubs them over the surface of the trough *b* for a sufficient length of time to thoroughly smooth, stiffen, and set the fibers and the coils. When 85 the coil has accumulated and has been rubbed and heated sufficiently, the feed-rollers are made to stop, and by a suitable contrivance the coil or bunch *g* is stripped off from the end of the spindle, and the feed-rollers and 90 chute are shifted back to the point for repeating the operation.

Crimped fiber lacks the permanency of the set, because in the crimping process the fibers cannot be retained long enough in contact with 95 the crimping-rolls to enable the heat and pressure to take sufficient effect. By the continuous action of the pressing, rubbing, and heating devices which this method affords, the product becomes essentially different from any 100

other, by the hardness and stiffness imparted to the fiber, stiffness of the coils, and especially the smoothed and polished surface of the fiber.

In practice the series of bunches or coils *g* are not wholly detached from each other, but remain more or less connected at the ends, although partial separation takes place. The bunches *g* may be baked or otherwise still further subjected to heat, if desired, after which they may be picked apart, as shown at *h*, Fig. 4, for use.

It will be seen that the coils are so nearly concentric in form that the fibers will pick apart in the most ready manner, enabling them

to be picked very rapidly and without damage to the fibers by hand.

What I claim, and desire to secure by Letters Patent, is—

Natural fibers of vegetable substances and animal-hair curled, heated, rubbed or ironed and thereby polished, and set or fixed in the curled form, as a new article of manufacture for upholstery purposes.

JOHN GEORGE STEPHENS.

Witnesses:

W. J. MORGAN,  
S. H. MORGAN.